

## UNITED STATES PATENT OFFICE

2,004,273

## PRODUCTION OF CELLULOSE DERIVATIVE PRODUCTS

Henry Dreyfus, London, England

No Drawing. Application July 22, 1931, Serial  
No. 552,546. In Great Britain July 30, 1930

8 Claims. (Cl. 18—54)

This invention relates to the production of filaments, yarns, threads, ribbons, films and other products from solutions of cellulose acetate or other cellulose esters or ethers.

5 According to the present invention solutions of cellulose acetate or other cellulose esters or ethers are spun into a liquid of such constitution that little or none of the solvent contained in the spinning solution is removed from the filaments or other formed products, or at least the filaments or other products on leaving the bath are liquid or substantially liquid. Preferably the cellulose acetate solution or solution of other ester or ether is extruded into a liquid 10 which is a non-solvent for the cellulose derivative and for the solvent of the spinning solution.

Water or aqueous liquids in general are very suitable for use in this preliminary step of the present invention in conjunction with solvents 20 in the spinning solution which are insoluble or substantially insoluble in water, for instance tetrachlorethane, chloroform, ethylene chloride, ethylene bromide, methylene chloride, and dichlorethylene. Such liquids are solvents for 25 some varieties of cellulose esters or ethers, or on the other hand become solvents with small additions of alcohols which will not substantially affect the solubility of the whole in water. Thus for instance methylene chloride, ethylene chloride and chloroform for certain varieties of cellulose acetate become solvents with very small 30 additions of methyl or ethyl alcohol. Where solvents are used in the spinning solutions which are miscible with water, their solubility or miscibility may be decreased by dissolving in the 35 aqueous bath calcium chloride, sodium acetate or other salts, preferably to a high concentration. In many cases, the water miscible solvents are insoluble in paraffin oil and like liquids so 40 that these may be used for this preliminary stage, especially when the spinning solution is made up with some water.

The present invention, does, however, include 45 the use of baths which will dissolve out some of the solvent in the spinning solution, but which nevertheless will leave the filaments or other products still in a liquid or substantially liquid state. For this purpose baths may be used which are to some extent solvents for the solvent in 50 the spinning solution, or alternatively additions may be made to the baths described above for the purpose of conferring upon them solvent properties for the solvent in the spinning solution. For instance to aqueous baths alcohols, 55 acetic acid or like acids may be added.

The bath used for the purpose of the present invention may differ somewhat in specific gravity from the spinning solution itself, so that the filaments or other products may rise or fall through the liquid in question, thus facilitating starting up. Alternatively or in addition the spinning may be started with a bath adapted to coagulate the spinning solution, and the bath characteristic of the present invention subsequently introduced so as to surround the spinning nozzle. Again when the subsequent setting of the filaments is to be effected by dry methods the spinning may be started up by any suitable method for dry spinning, and the bath subsequently introduced as before.

The length of the preliminary bath of water, hydrocarbon or other liquid in which the filaments or other products are formed may vary very widely. It depends to some extent upon the amount of "draw-down", if any, which is applied 20 to the filaments or other products and also upon the viscosity of the spinning solution. In most cases a length up to a few inches suffices to produce the advantages of the present invention.

The filaments or other products, which will 25 be of substantially the same composition as that of the original spinning solution or only have comparatively small amounts of solvent abstracted therefrom so that they are still liquid, may be solidified by dry or wet methods 30 or by a combination of the two. In the case of many of the wet methods it is of advantage as described in U. S. Patents Nos. 1,465,994 and 1,467,493 and British Patents Nos. 340,324, 340,325 and 343,062 to employ in the coagulating bath a solvent for the cellulose derivative 35 so as to produce strong filaments or other products. Where feasible the coagulating bath may be used contiguously with the preliminary bath of the present invention. For instance one 40 may be floated on the other and the filaments caused to pass up or down through the two layers of bath. Again the filaments or other products may be solidified by dry spinning methods, in which case they should rise or be 45 drawn up through the preliminary bath characteristic of the invention. For example the preliminary bath may be placed at the bottom of an upward dry spinning cell so that the filaments pass up through the liquid and are 50 then drawn up through the cell through which may be passed an evaporative medium and are finally either wound at the top or taken out of the cell and afterwards wound. The conditions obtaining in the dry spinning cell may 55

be such as to produce any type of product, for example products of round cross-section and of dull high lustre.

Again coagulating baths consisting of or containing mineral acids or mineral acid esters or organo mineral acids, e. g. sulphonic acids, may be employed, as described in U. S. Patents Nos. 1,903,299 and 1,950,024.

The filaments or other products solidified by dry or wet methods may be passed round a feed roller or other device adapted to apply tension thereto, and in fact it is found that, by reason of the method of formation, the filaments or other products can be drawn out to produce very fine deniers or low cross-sections. The invention is however not limited to the production of such fine products, since it presents advantages even when comparatively large filaments, such as may be used for horse-hair or bristles, are produced, such products having improved extensibility and tenacity.

The following examples illustrate the invention, but they are not to be considered as limiting it in any way:

#### Example 1

An acetone soluble cellulose acetate, preferably of relatively high acetyl content, as for example 56-57% (calculated as acetic acid), which may be produced for example as described in my British Patent No. 309,201, is dissolved in tetrachlorethane so as to form a 20-25% solution. In the event that complete solution does not occur, a small amount of alcohol may be added thereto so as to promote solution. The said spinning solution is then spun as follows:—A coagulating bath provided with a partition across the full width thereof, but not reaching to the bottom, is filled with tricresyl phosphate up to above the level of the spinning nozzle which is adapted to spin downwards. The partition may advantageously reach to a point some three inches below the level of the spinning nozzle. Below the partition and towards the bottom of the bath is provided a suitable guide or other member round which the filaments may be passed. Spinning is then started up in the customary manner, the filaments being carried round a guide under the partition and up out of the bath through the compartment not containing the spinning nozzle. Water is then carefully run into the compartment containing the spinning nozzle until its lower level is at a point about 1 to 2 inches below the spinning nozzle. The spinning may thereafter be run continuously. After leaving the bath the filaments may be carried round a suitable feed roller adapted to draw them out to the required denier. As already indicated the process of the present invention is especially adapted to produce products of very low denier indeed. On leaving the feed roller the filaments may be collected in a centrifugal box or may be wound or twisted and wound in any other desired manner. The tricresyl phosphate may then be extracted from the yarn with the aid of benzene or any other suitable agent. The products obtained have a high resistance to the action of hot aqueous liquids.

#### Example 2

A coagulating bath containing a spinning nozzle adapted to spin upwardly is provided with a coagulating liquor consisting of 50% of petro-

leum spirit, having a boiling point of 60-120° C. and 50% of ethylene dichloride. A 20-25% spinning solution of an acetone soluble cellulose acetate is then made up in ethylene dichloride containing a small amount of alcohol. Spinning is then started up in the usual manner, and after the filaments have been carried round the customary feed roller a saturated aqueous solution of common salt is run slowly and carefully into the bottom of the bath, as for example by means of a tube or pipe reaching to the bottom, until the spinning nozzle is immersed therein to a depth of 1 to 2 inches. Spinning is thereafter carried on continuously, and the filaments may, as described in Example 1, be stretched and collected in any suitable manner. As in Example 1 they may, while being wound or twisted and wound, be washed with benzene or with petroleum spirit.

#### Example 3

Spinning is conducted in the apparatus described with reference to Figure 2 in British Patent No. 351,718. The cup described therein is provided with an overflow at a level of 1 to 2 inches above the face of the spinning nozzle. Initially the cup is filled up to the level of the overflow with benzene or petroleum ether. Spinning is started up as described in the said British patent, using a spinning solution prepared according to Example 2 above, the filaments being set by a dry spinning process after passage through the hydrocarbon layer. Once spinning has started up water is run in to the cup until the benzene or petroleum hydrocarbon has been completely displaced. Spinning is then continued in the manner customary in dry spinning processes. As before the filaments may be drawn out to very fine deniers. They may be wound or twisted and wound, as for example by a cap spinning device.

The filaments or other products produced according to any of the above methods may be further treated in any desired manner to impart improved properties thereto. For instance they may be stretched when in the finished condition, whether or not they have been drawn out or stretched during the formation, so as to obtain still further increased strength. Again they may be treated according to the process described in my British Patent No. 359,971 with or without stretching. This specification describes impregnating the materials with relatively dilute solutions of solvents or softening agents and subsequently concentrating the solutions on the material so as to enable them to exert a solvent action thereon. Examples of suitable solvents or softening agents are aqueous solutions of thiocyanates, such as those of the alkalies, ammonium and alkaline earths, aqueous solutions of zinc chloride, acetic acid, formic acid, lactic acid, diacetone alcohol, methyl or ethyl lactate, acetone, and the like; and mono- and di-ethers or esters or ether esters of olefine glycols and poly-olefine glycols, for instance the mono- and di-methyl and ethyl ethers of ethylene glycol, glycol mono-acetate, methyl glycol acetate, dioxane, the mono-methyl and ethyl ethers of propylene glycol, and the mono-ethyl ether of diethylene glycol etc.; phenols, formaldehyde, acetaldehyde, mono-, di- and tri-acetins, dichlorethylene, and the like, mineral acids, sulphonic or other organo mineral acids, or acid esters of mineral acids, or mixtures of these, or solvent mixtures. The

agent with which the filaments or threads are treated may be diluted with a liquid or diluent which is not a solvent of the cellulose derivative, for instance water, benzene or the like. 5 The solvent action may be exerted on the filaments or other products with or without simultaneous stretching.

The invention is broadly applicable to the production of filaments, threads, and other products etc. from solutions of any suitable cellulose derivatives, for example cellulose acetate or other carboxylic acid esters of cellulose, e. g. cellulose acetate, formate, propionate, butyrate and the like or other esters of cellulose, e. g. cellulose nitrate, and cellulose ethers, for instance methyl, ethyl or benzyl cellulose.

What I claim and desire to secure by Letters Patent is:—

1. Process for the manufacture of filaments, 20 yarns, threads, ribbons, films and like products from solutions of organic derivatives of cellulose, comprising extruding said solutions into a liquid which is a non-solvent for the organic derivative of cellulose and is substantially a 25 non-solvent for the solvent in the organic derivative of cellulose solution, and then leading the products from said liquid whilst they are still substantially liquid, into a setting medium.

2. Process for the manufacture of filaments, 30 yarns, threads, ribbons, films and like products from solutions of cellulose acetate, comprising extruding said solutions into a liquid which is

a non-solvent for the cellulose acetate and is substantially a non-solvent for the solvent in the cellulose acetate solution, and then leading the products from said liquid whilst they are still substantially liquid, into a setting medium. 5

3. Process for the manufacture of filaments, 10 yarns, threads, ribbons, films and like products from solutions of cellulose acetate, comprising extruding solutions of the cellulose acetate in solvents substantially immiscible with water 10 into water, and then leading the same from the water while the products are still substantially liquid into a setting medium.

4. Process according to claim 1, wherein the 15 organic derivative of cellulose solution is caused to pass through the liquid for a comparatively short distance on the order of 1 to 2 inches.

5. Process according to claim 1, wherein the 20 setting of the products is effected by wet spinning processes.

6. Process according to claim 2, wherein the 25 setting of the products is effected by means of coagulating baths comprising a proportion of solvent for the cellulose acetate.

7. Process according to claim 1, wherein the 30 setting of the products is effected by dry spinning processes.

8. Process according to claim 1, wherein the products are drawn down to products of low 35 denier or small cross-section.

HENRY DREYFUS.